

**[54] LOW TEMPERATURE GAS GENERATOR PROPELLANT****[75] Inventor:** **Eugene F. Garner**, Saugus, Calif.**[73] Assignee:** **Allied Chemical Corporation**, New York, N.Y.**[22] Filed:** **Aug. 26, 1974****[21] Appl. No.:** **500,810****Related U.S. Application Data****[63] Continuation-in-part of Ser. No. 395,481, Sept. 10, 1973, Pat. No. 3,901,747.****[52] U.S. Cl. ....** **149/41**; 149/41; 149/42; 149/43; 149/46; 149/76; 149/75; 149/82**[51] Int. Cl.<sup>2</sup>.....** **C06B 33/14****[58] Field of Search** .... 149/40, 41, 42, 43, 46, 149/61, 76, 82; 252/188.3 R**[56] References Cited****UNITED STATES PATENTS**

3,647,393 3/1972 Leising et al. .... 102/39 X

*Primary Examiner—Stephen J. Lechert, Jr.  
Attorney, Agent, or Firm—Jonathan Plaut***[57]****ABSTRACT**

This pyrotechnic composition is adapted, upon combustion, for generating a low-flame temperature, non-toxic gas for inflating a vehicle safety bag or other inflatable device. The composition comprises: a fuel, such as a carbonaceous material, aluminum or magnesium; an inorganic oxidizer, such as a metal chlorate, a metal perchlorate, a metal nitrate, ammonium chlorate, ammonium perchlorate or ammonium nitrate; and a coolant or combined binder and coolant, such as magnesium carbonate, magnesium hydroxide or a mixture of magnesium hydroxide and magnesium carbonate. A typical example of this composition comprises: carbon as the fuel; potassium chlorate as the oxidizer; and magnesium carbonate or a mixture of magnesium hydroxide and magnesium carbonate as the binder-coolant. One may use as much of this later mentioned binder-coolant as is necessary to obtain the desired binding properties in the composition, without raising the flame temperature of the gas to an unacceptable level.

**7 Claims, No Drawings**

## LOW TEMPERATURE GAS GENERATOR PROPELLANT

### CROSS-REFERENCE TO RELATED APPLICATION

This application is a continuation-in-part application of my previous patent application Ser. No. 395,481, filed September 10, 1973, now U.S. Pat. 3,901,747 entitled "Pyrotechnic Composition With Combined Binder-Coolant".

### BACKGROUND OF THE INVENTION

This invention relates to a pyrotechnic composition adapted, upon combustion, for generating gas. In particular, this invention relates to a pyrotechnic composition which, upon combustion, generates a low temperature, non-toxic gas. Among the uses for such a gas is to inflate a safety bag in a vehicle to restrain movement of an occupant in the vehicle in the event of collision, or in the case of slower burning mixtures, to be defined in one embodiment later, producing gas with a relatively low temperature, the substantially non-toxic gas produced may be used to inflate life rafts, emergency airline slides, buoys, tires or other inflatable devices.

It is necessary that pyrotechnic compositions be able to meet certain criteria in order to be adapted for use with a vehicle safety air bag restraint or other such inflatable devices. The pyrotechnic composition must be able to withstand storage in an environment from approximately -40°F. to approximately +220°F. For the vehicle safety air bag applications, it is also necessary that the composition be capable of being ignited rapidly, for example, within a matter of milliseconds, and that it be capable of being totally ignited to produce gas. In some other applications, a slow burn is not a disadvantage and a relatively cool gas is highly advantageous, as will be discussed. It is necessary that the gas produced have only a negligible amount of toxic gases, such as nitrogen oxides or carbon monoxide.

Previously used pyrotechnic compositions normally include the use of an organic binder. The organic binder also acts as a fuel and tends to raise the flame temperature of the gas to an unacceptable level. As a result, the temperature of the outer surface of the vehicle safety bag or other inflatable device, using such prior art compositions, would be so high that it might burn the user.

This is understandable because the compositions using such binders were intended for applications such as high-energy propellants for rockets, where low temperature was not an objective. See: U.S. Pat. Nos. 2,929,697 to Perry and 2,994,598 to Dickey. In addition, many of the compositions disclosed in the prior art produce a toxic gas, such as some of the compositions in U.S. Pat. Nos. 3,020,180 to Morello and 3,047,524 to Bowman.

### SUMMARY OF THE INVENTION

The pyrotechnic composition of this invention is adapted, upon combustion, for generating a low temperature, substantially non-toxic gas for the application desired. This gas is useful for inflating various devices, such as a safety bag in a vehicle. A safety bag is inflated to restrain the movement of an occupant of the vehicle in the event of collision. Where a composition producing a low temperature gas from a relatively slow burn is utilized, as will be discussed later, application to other already mentioned inflatable devices is advanta-

geous. In general, the pyrotechnic composition comprises a fuel; an inorganic oxidizer; and a coolant or combined binder and coolant (which also is referred to as just a coolant in the following description), which is selected from the group consisting of magnesium hydroxide, magnesium carbonate, and a mixture of magnesium carbonate and magnesium hydroxide. It has been found that one may use as much of the binder-coolant as is necessary in the pyrotechnic composition to obtain the desired binder properties for the composition without raising the flame temperature of the gas, generated upon combustion, to an unacceptable level. The fuel may be selected from the group consisting of: a carbonaceous material, aluminum and magnesium. The inorganic oxidizer may be selected from the group consisting of: a metal chlorate, a metal perchlorate, a metal nitrite, ammonium chlorate, ammonium perchlorate, and ammonium nitrite.

### DETAILED DESCRIPTION

This pyrotechnic composition is adapted for generating a low temperature, non-toxic gas upon combustion for inflating a vehicle safety bag or other inflatable device. In general, the composition comprises: a fuel selected from the group consisting of a carbonaceous material (such as carbon, carbon black or lamp black), aluminum and magnesium; an inorganic oxidizer selected from the group consisting of an alkali metal chlorate, such as potassium chlorate or sodium chlorate, an alkali metal perchlorate, such as potassium perchlorate or sodium perchlorate, an alkali metal nitrate, such as potassium nitrate or sodium nitrate, ammonium chlorate, ammonium perchlorate, and ammonium nitrate; and a coolant or combined binder and coolant selected from the group consisting of: magnesium carbonate, magnesium hydroxide, and a mixture of magnesium carbonate and magnesium hydroxide. A typical formulation of this pyrotechnic composition comprises: carbon which acts as a fuel; potassium chlorate ( $KClO_3$ ) or potassium perchlorate ( $KClO_4$ ) which acts as an oxidizer; and a magnesium carbonate ( $MgCO_3$ ) and magnesium hydroxide ( $MgOH_2$ ) mixture which acts as a coolant and binder.

In the case of the composition of carbonaceous fuel, inorganic oxidizer and magnesium carbonate coolant, a low temperature gas (about 800°F in one embodiment) is generated relatively slowly (in, for example, about 1 to 3 seconds) which may be cooled, as by contact with a metal chip bed, to a temperature of from 200°F. to 600°F., for inflating an inflatable device such as a life raft, inflatable buoy, tire, emergency slide, etc., which may then be in contact with the user.

The pyrotechnic composition of this invention comprises by weight: from less than 1% to about 10% of one of the foregoing fuels, such as carbon; from about 30% to about 70% of one of the foregoing inorganic oxidizers, such as potassium chlorate; and from about 10% to about 60% of one of the foregoing coolants or combined binders and coolants, such as magnesium carbonate or a mixture of magnesium carbonate and magnesium hydroxide.

Preferably, in one embodiment, the pyrotechnic composition comprises by weight: about 3% to about 7% of one of the foregoing fuels, such as carbon; about 40% to about 60% of one of the foregoing inorganic oxidizers, such as potassium chlorate; and about 35% to about 55% of one of the foregoing combined binders

and coolants, such as a mixture of magnesium hydroxide and magnesium carbonate. When such compositions are burned in the presence of air, the magnesium hydroxide reacts with carbon dioxide ( $\text{CO}_2$ ) in the air to form magnesium carbonate ( $\text{MgCO}_3$ ). Magnesium carbonate is a highly oxygenated, cement-like material and, by itself, provides no binding properties. The conversion of magnesium hydroxide to magnesium carbonate provides the binding effect. Neither the magnesium hydroxide nor the magnesium carbonate acts as a fuel. Since magnesium hydroxide and magnesium carbonate are both coolants, not fuels, one can use as much as necessary. As a result, one has enough binder for the composition without raising the flame temperature of the gas to unacceptable levels. The free oxygen formed from the inorganic oxidizer, such as potassium perchlorate, is consumed by the fuel, such as carbon, forming carbon dioxide and evolving heat which is cooled by the magnesium hydroxide.

In this last mentioned embodiment (in the preceding paragraph) it is preferable, in most instances, to start with a mixture of magnesium hydroxide and magnesium carbonate, rather than magnesium hydroxide without magnesium carbonate. One should use enough magnesium hydroxide in the mixture to obtain the desired binding effect caused by the carbonation of the magnesium hydroxide. But, one should use only enough magnesium hydroxide to obtain the necessary physical properties as a binder because in compositions using a mixture of magnesium hydroxide and magnesium carbonate, it has been found that the higher the proportion of magnesium hydroxide to magnesium carbonate that is used in the composition, the longer the reaction time will take.

More specifically, in this last discussed embodiment, the magnesium hydroxide in the pyrotechnic composition should comprise by weight not less than about 10% of the entire composition and preferably from about 10% to about 30% of the entire composition. In instances where a mixture of magnesium hydroxide and magnesium carbonate is used as the combined binder and coolant, the composition may comprise: from about 10% to about 30% magnesium hydroxide as compared to the entire composition and from about 20% to about 40% magnesium carbonate as compared to the entire composition. In many compositions it has been found advantageous for the mixture of magnesium hydroxide and magnesium carbonate to comprise about one-half magnesium hydroxide and about one-half magnesium carbonate.

In the preferred embodiment previously mentioned (carbon fuel, potassium chloride or perchlorate oxidizer, and magnesium carbonate coolant) where a relatively low burning composition produces a relatively low temperature gas (which may optionally be further cooled as already discussed), it has been surprisingly found that the magnesium carbonate burns in the presence of the oxidizer and the carbon fuel to support the combustion at a very high temperature, but relatively slowly, with the magnesium carbonate decomposing to absorb the heat and produce the relatively low temperature gas product made up of, substantially, carbon dioxide ( $\text{CO}_2$ ) and oxygen, with trace amounts of carbon monoxide ( $\text{CO}$ ).

The following examples, in which percent is by weight, are provided for purposes of illustration.

5 The composition used comprises: 5% carbon as the fuel, 50% potassium chloride as the inorganic oxidizer, and 45% of a mixture of magnesium hydroxide and magnesium carbonate as the binder-coolant. The proportion of this mixture was approximately one-half magnesium hydroxide and one-half magnesium carbonate so that the magnesium hydroxide and the magnesium carbonate each formed 22-178% of the total composition.

#### EXAMPLE 2

15 The composition comprised: 5% carbon, 50% potassium chloride; and 45% magnesium hydroxide.

#### EXAMPLE 3

20 The composition comprised: 5% carbon, 51% potassium chloride; and 44% magnesium hydroxide.

#### EXAMPLE 4

25 The composition comprised: 6% carbon; 50% potassium chloride; and 44% magnesium hydroxide.

25 The compositions in the foregoing examples each produce a gas having a flame temperature from about 1500°F. to less than 2000°F.

30 The pyrotechnic compositions above of this invention achieve flexibility in reference to the amount of binder which may be used, consistent with the object of producing a gas having a low-flame temperature and a negligible amount of toxic gases, such as nitrogen oxides or carbon monoxide.

#### EXAMPLE 5

35 The composition comprised: 3% carbon as the fuel; 45% potassium chloride as the inorganic oxidizer; and 52% magnesium carbonate as the coolant.

40 It has been found useful in one embodiment to pelletize the pyrotechnic composition of this invention in order to achieve a predictable combustion performance of the composition, rather than to use the composition in powder form. Pelletizing can be achieved by severely mixing the powdered ingredients and then using a pill press to produce pellets, or by granulating the powdered mixture, extruding it through a screen and forming noodles. Pelletizing has been found advantageous because of the following undesirable characteristics of a mixed powder. The powder tends to separate, with the oxidizer at the bottom and the fuel at the top. When the powder burns, it burns with different characteristics depending upon the degree to which the powder mixture is homogeneous. In addition, the powder may be loosely packed or it may become tightly packed which also affects its burning or combustion characteristics. The result is that inconsistent results are sometimes obtained when using the composition in powder form. When using the composition in pellet form, more consistent results are generally produced. Optionally, an organic lubricant, such as stearic acid or Carbowax (a trade name of Union Carbide Corporation for polyethylene glycols), may be added to pelletizing.

45 I claim:

50 1. A pyrotechnic composition adapted, upon combustion, for generating a low temperature, substantially non-toxic gas, said composition comprising: a fuel selected from the group consisting of a carbonaceous ma-

terial, aluminum and magnesium; an inorganic oxidizer selected from the group consisting of a metal chlorate, a metal perchlorate, a metal nitrate, ammonium nitrate, ammonium chlorate, and ammonium perchlorate; and a coolant selected from the group consisting of magnesium hydroxide and a mixture of magnesium carbonate and magnesium hydroxide.

2. The pyrotechnic composition according to claim 1 comprising by weight: about 1% to about 10% of said fuel; about 30% to about 70% of said inorganic oxidizer; and about 10% to about 60% of said coolant.

3. The pyrotechnic composition according to claim 1 comprising by weight: about 3% to about 7% of said fuel; about 40% to about 60% of said inorganic oxidizer; and about 35% to about 55% of said coolant.

4. The pyrotechnic composition according to claim 1 wherein said magnesium hydroxide comprises by

weight about 10% to about 30% of the entire composition.

5. The pyrotechnic composition according to claim 1, wherein said coolant comprises about 10% to about 30% magnesium hydroxide as compared to the entire composition and about 20% to about 40% magnesium carbonate as compared to the entire composition.

6. The pyrotechnic composition according to claim 5 wherein said mixture of magnesium hydroxide and magnesium carbonate comprises about equal amounts of magnesium hydroxide and magnesium carbonate.

7. The composition according to claim 1 comprising by weight: 5% carbon; about 50% potassium chlorate; and about 45% of a mixture of about equal amounts of magnesium hydroxide and magnesium carbonate.

\* \* \* \* \*

20

25

30

35

40

45

50

55

60

65

### **Disclaimer**

3,912,562.—*Eugene F. Garner, Saugus, Calif.* LOW TEMPERATURE GAS GENERATOR PROPELLANT. Patent dated Oct. 14, 1975. Disclaimer filed Feb. 22, 1977, by the assignee, *Allied Chemical Corporation*.

The term of this patent subsequent to Aug. 26, 1992, has been disclaimed.  
[*Official Gazette May 3, 1977.*]